

Sept. 1, 1936.

E. R. POWELL

2,052,842

EXPANDING MASONRY

Original Filed June 29, 1932

2 Sheets-Sheet 1



INVENTOR.

Edward R. Powell.

Sept. 1, 1936.

E. R. POWELL

2,052,842

EXPANDING MASONRY

Original Filed June 29, 1932 2 Sheets-Sheet 2

37

*Fig. 6.*



*Fig. 7.*

34

36

38 30



INVENTOR.

*Edward R. Powell.*

Patented Sept. 1, 1936

2,052,842

# UNITED STATES PATENT OFFICE

2,052,842

## EXPANDED MASONRY

Edward R. Powell, Alexandria, Ind.

Application June 29, 1932, Serial No. 619,845  
Renewed July 20, 1935

26 Claims. (Cl. 72—1)

This invention relates to a form of masonry which uses expanded building units as the principal material.

It relates particularly to a form of masonry structure in which light-weight ceramic building units are employed. One of the principal features of the invention is the use of these light-weight units to form a structure which is more rugged and will support a larger volume of itself than common masonry. In this form of masonry, the density (and to some extent the strength) of the building units is proportioned to the function which the units perform in the structure. That is, for example, a tile which forms a panel wall and acts as only a windbreak will, in general, have the lowest density; while one which is part of the compression fiber of a beam or one of the lower load bearing columns will ordinarily have the highest density and, in general, the highest strength. Other functions in the structure may be performed by units of intermediate strength or density.

Another feature of the invention consists in using reinforcement such as steel rods to lend stability to the lighter parts of the structure and permit the construction of beams and other composite members in which the rods supply the tensile strength necessary to sustain the stresses on the structure.

The object of the invention is to build a structure which has the advantages of reinforced concrete without the use of forms, and which has the additional advantages of having permanent decorative faces and better heat insulating and sound absorbing properties. Another object is to provide a structure which has minimum weight for its strength, considering the class of materials which it employs.

The full nature of the invention will be understood more readily by reference to the accompanying drawings and the following description and claims.

In the drawings:

Fig. 1 is an elevation of part of a building which embodies the invention, the nature of the masonry in various parts being illustrated by symbols which will be explained hereinafter.

Fig. 2 is an enlarged sectional detail of one means of anchoring a reinforcing rod in the masonry.

Fig. 3 is an enlarged sectional detail of a modified form or anchor for tie rod or reinforcing rod.

Fig. 4 is a section of part of the structure of

Fig. 1 taken on the plane 4—4 and in the direction of the arrows.

Fig. 5 is a section of part of the structure of Fig. 1 taken in the plane 5—5 and in the direction of the arrows.

Fig. 6 is a vertical section of a slab such as a floor or roof slab built of reinforced variably expanded masonry.

Fig. 7 is an enlarged section taken on line 7—7 of Fig. 6 in either direction.

In the drawings, the areas rendered in dots only are surfaces of material of maximum strength; those rendered in relatively large circles only are the weaker and usually much lighter materials. The surfaces of materials of intermediate strength or density are indicated by both dots and circles.

These expanded building units may be made by expanding clay in the pyro-plastic condition as described in my application Serial No. 522,272 now Patent No. 1,963,029, or expanded in wet liquid condition as described in my applications Serial Nos. 600,115 and 601,796 now Patent Nos. 1,963,030 and 1,963,031, respectively, or it may be made by any other process which produces expanded material in units which are suitable for structural purposes.

In Fig. 1, 11 designates a footing or foundation which supports part of the building. A column 32 rests on this footing and is reinforced by rod 12. A panel wall 13 is adjacent to the column 32. There are plates such as 15 on the ends of the rod 12. A continuation of column 32 is designated by 14 with similar rod 12 and panel wall 13. The part of the column 14 is lighter than the portion 32. Another portion 16 is lighter than 14. The panel walls 13 are all about the same density because they carry only themselves between stories. At the top of portion 16, the column portion joins a typical beam portion. The rods 19 and 20 take the tension on the lower fiber of the beam. The upper portion of the beam 28 which is in compression is of high strength material; while the lower portion 18 which acts as a protection for the rods and fills in the structure may be of lower strength. The rods 19 and 20 have anchor plates such as 21 to distribute the tension. The beam supports a portion 17 of a panel wall.

In Fig. 2, the relatively heavy rod 33 is embedded in the masonry. It is embedded more particularly in the mortar 30 which is the bonding material between the units. The mortar is ordinarily lime, Portland cement and sand. For a very hard mortar, two parts of Portland cement may

be used to one of lime and nine parts of sand. The proportion of sand will vary with the nature of the sand particle size and how well it packs. Both the sand and the water are usually proportioned on the job to give a mortar of proper working consistency. The mortar may be all Portland cement, it may be gypsum plaster, magnesium oxy-chloride cement, asphaltic mixtures or any other material suitable for bonding building units provided the service which is involved permits the use of these materials.

The rod may be laid in a channel provided for same in the units, it may be laid by notching the units, or the mortar joints may simply be made thick enough to enclose the rods. In any case the final structure consists of units firmly bonded together by means of a mortar in which a rod is at least partly embedded. The rod 33 is preferably rolled with rough or cleated surfaces so that it will be firmly gripped by the hardened mortar. The rod 33 is provided with a nut 23 which bears against the plate 22 so as to distribute the load over enough of the masonry to avoid local crushing. The plate may be slightly dished or channelled to provide a little spring. This tends to prevent crushing and will take up a little difference in expansion between the rod and the rest of the structure. The units 29 adjacent to the plate are shown of intermediate strength.

Fig. 3 shows another form of anchor in which the rod 25 has a hooked portion 31 which connects with a heavier cross rod 24. The rod 25 is preferably a commercial reinforcing rod such as used for concrete reinforcement. It is embedded in the bonding material. The units in Fig. 3 are shown of intermediate strength also.

The expanded ceramic material which has been developed for such service may have nearly as much strength as solid masonry and still be considerably lighter. The expanded material usually has much better bonding properties than regular brick or hollow tile so that the structure as a whole may be stronger than masonry of conventional type. The better bonding properties of the expanded units result principally from the enclosed gas-formed cells which are partly exposed on the surface so that the mortar penetrates an appreciable distance into the units in places and "keys" itself thereto.

Fig. 4 shows a portion of the beam and adjacent panel walls. The portion of the beam shown is under mainly shearing stress which the intermediate strength material will stand. It is under some compression stress also from the tension of the rods. In Fig. 5, however, which is near the middle of the span, the upper part of the beam is under considerable compression stress while the lower portion is under tension. The rods, of course take the tension so that the masonry proper is under very little stress. Lighter material is therefore used in this portion of the beam. The units of which the beam is built are shown specially designed to interlock and provide channels for the rods 19 and 20. There is a sloping sill 26. Similar results may be obtained by using standardized size and shape units by using a little more mortar and bonding it well to the units. Most water-mixed mortars will bond better to the units if the unit surface is wet. An additional load which may be carried by the beam is shown in dotted lines. The inner wall 17 may have a decorative coating of some sort.

Fig. 6 shows a slab suitable for a floor or roof. The units 34 are understood to be of different character in different parts. That is they have

a variation in the degree or character of the expansion within themselves. For example, the upper part may reach a maximum density of 75 lb. per cu. ft. while the lower part may have a minimum density of 25 lb. per cu. ft. The units as shown are provided with channels 36 which admit the reinforcing rods 38. The rods 38 terminate preferably in plates 37 which may be welded on or held with nuts or threads. For large areas, the slabs are sometimes supported on steel T-irons 35 or other structural members. In this case, the rods may be secured to the web of the T-iron instead of to separate plates.

A sub-floor of Portland cement mortar may be poured on the slab and a composition floor laid over this. For roof service a built up roofing may be used and composition service floor over the roofing. The sub-floor 39 should be well bonded to the units 34, wetting the units if necessary. The lower surface of the units 34 may be decorative and be of "open" structure so as to have acoustical properties. The construction of a slab of this sort usually requires false work which should be left in place until the mortar has set and hardened. The false work may, if desired, be supported from the T-irons.

In general the pyro-plastically expanded ceramic material permits lower density without sacrifice of strength. That is brick of practically full strength have been made by pyro-plastic expansion at 35 lb. per cu. ft. density. At a sacrifice of strength, the density may be as low as 18 to 20 lbs. per cu. ft. The wet plastic material usually has less strength for a given density but is easier to produce by certain processes in special shapes and textures. Typical densities for the various parts of the structure of Fig. 1 for the wet expanded material may be as follows: Part 11, 100 lbs. per cu. ft.; part 32, 75 lbs.; part 14, 65 lbs.; part 16, 55 lbs.; part 13, 35 lbs.

Expanded masonry may be of constant density or it may not be reinforced. While a specific group of structures is illustrated, it should be understood that any masonry structure where the listed advantages are desired may ordinarily be designed on the same principles. In general, the invention is involved in any structure in which the density of the structural units is reduced in places to lighten the structure and improve its properties, the difference in density being secured by cellular expansion of the material. The above examples should therefore be taken as illustrations and not in a limiting sense.

Structural ceramic material is intended to include preformed structures which are formed by the application of heat to clayey material of plentiful grade. These may or may not be of refractory type but must be load bearing where loads are imposed and weather resistant where exposed. Usually refractory materials are resistant to high temperatures but, if expanded at all, will not carry loads or stand the weather.

The invention claimed is:

1. In a composite building structure, the combination of a relatively hard and relatively high bonding strength mortar in continuous frame work arrangement, relatively high tensile strength reinforcing material imbedded in said frame work, and a plurality of independent structural units united by said frame work and each including a relative dense portion and a cellular or open work portion.

2. A single course wall like reinforced masonry structure adapted to resist bending moment which includes a plurality of originally inde-

pendent, cellular expanded masonry units, jointing mortar in unitary frame work arrangement for securing the units together, reenforcing means for the wall structure and included in the jointing mortar, substantially all units having a cellular portion of relatively high thermal insulating value, certain of said cellular masonry units having another and relatively denser portion resistant to high compression stress, said units being so arranged in said wall that the denser portion will be positioned to prevent rupture in the cellular portions as a wall when subjected to high compression strength, the thermal resistance of the entire wall being approximately the same as that of the individual units when measured in the same direction.

3. A structure as defined by claim 2, characterized by each cellular unit having its cellular portion provided with an open type surface for acoustical purposes in addition to the insulating thermal resistance.

4. A building structure of expanded character, including in combination a plurality of building units each of expanded character and having relatively low mechanical strength and high thermal insulating value compared with standard building units of like dimension and like original material, said expanded units being arranged in unitary formation, relatively hard bonding material between said units for securing the same in said formation and constituting a unitary frame work, and relatively high tensile strength reenforcing material imbedded in the bonding material frame work, said relatively hard bonding material having a relatively high bonding relation with the low mechanical strength units to supplement the strength of said units when in structural formation.

5. A reenforced masonry structure adapted to resist bending moment which includes a plurality of cellular expanded units, mortar for securing said units together, said mortar forming a unitary frame work for said units and having relatively high strength and hard bonding power with said units, certain of said expanded units each having different degrees of expansion in different portions of said unit, whereby a portion in each unit has a relatively great crushing strength for accommodating principal compressive stresses, and another portion of said unit has less crushing strength and of higher thermal insulating value, said last mentioned portion not being subjected to the principal compressive stresses, said units being arranged in the structural formation so that the said portions have the accommodation value specified, and reenforcing means for the structure and enclosed in the mortar frame work.

6. A multiple course reinforced masonry structure adapted to resist bending moment which includes a plurality of cellular expanded units arranged in courses, mortar for securing said units together, said mortar forming a unitary frame work for said units and having relatively high strength and hard bonding power with said units, most of the units in different courses having different degrees of expansion, some units having a relatively great crushing strength for accommodating principal compressive stresses, and other units having less crushing strength and of higher thermal insulating value, said last mentioned units not being subject to the principal compressive stresses, said units being arranged in the structural formation so that the said units have the accommodation value speci-

fied, and reinforcing means for the structure and enclosed in the mortar frame work.

7. A structure as defined by claim 1 which has, when subjected to bending moment, certain regions of high compressive stress and certain regions of high tensile stress, the high compressive stress regions consisting of the hard mortar and the dense portions of the units; and the high tensile stress portions consisting of the hard mortar, and the reinforcement of the cellular portions of the units.

8. In a composite building structure, the combination of a relatively hard and relatively high bonding strength mortar in continuous frame work arrangement, relatively high tensile strength reinforcing material imbedded in said frame work, and a plurality of independent structural units united by said frame work and each including a portion of relatively high thermal resistance, the thermal resistance of the whole structure being approximately equal to that of the individual units when measured in the same direction.

9. A ceramic structural unit comprising a true ceramic material of relatively high density and a light weight cellular layer inseparably united with one of the surfaces of said body portion, the relative thickness of the dense and cellular bodies being varied in accordance with conditions or service to which the material is placed, said cellular material being of substantially uniform composition throughout and characterized by the inclusion throughout its body of separate and closed cells separated by thin cell walls of true ceramic material.

10. As a new article of manufacture, a structural unit comprising a body portion of relatively high density, and a heat insulating portion composed of a cellular argillaceous material inseparably united with said body portion, said cellular material comprising a heat-treated argillaceous body of substantially uniform composition throughout and of predetermined shape and dimensions, and characterized by the inclusion throughout its body of separate and closed cells separated by relatively thin cell walls of fired-clay material having in its unit form a density of less than one-half the density of the first-named body portion of said unit.

11. A ceramic or refractory unit comprising a structural material of relatively high density and a light weight cellular layer inseparably united with one of the surfaces of said refractory material of high density, the relative thickness of the dense and cellular materials being varied in accordance with conditions of service to which the unit is placed, said cellular material being of substantially uniform composition throughout and characterized by the inclusion throughout its body of separate and closed cells separated by thin cell walls of true ceramic material.

12. A ceramic structure comprising a ceramic material of relatively high density and an integrally attached adjoining layer of heat-insulating ceramic material, said heat-insulating material being of substantially uniform composition and characterized by inclusion throughout its body of separate cells separated by thin walls of ceramic material.

13. As a new article of manufacture, a structural unit comprising a body portion of relatively high density, and a heat insulating portion composed of a cellular material inseparably united with said body portion, said cellular material comprising a body of substantially uniform com-

position throughout and of predetermined shape and dimensions, and characterized by the inclusion throughout its body of separate and closed cells separated by relatively thin cell walls of material having in its unit form a density of less than one-half the density of the first-named body portion of said unit.

14. As a new article of manufacture, a structural ceramic unit comprising a body portion of relatively high density, and a heat insulating portion composed of a cellular material inseparably united with said body portion, said cellular material comprising a body of substantially uniform composition throughout and of predetermined shape and dimensions, and characterized by the inclusion throughout its body of separate and closed cells separated by relatively thin cell walls of material having in its unit form a density of less than one-half the density of the first-named body portion of said unit.
15. A structural unit as defined by claim 9, characterized by the inseparable union being an

integral formation with the remainder of the unit.

16. A structural unit as defined by claim 10, characterized by the inseparable union being an integral formation with the remainder of the unit.

17. A structural unit as defined by claim 11, characterized by the inseparable union being an integral formation with the remainder of the unit.

18. A structural unit as defined by claim 12, characterized by the inseparable union being an integral formation with the remainder of the unit.

19. A structural unit as defined by claim 13, characterized by the inseparable union being an integral formation with the remainder of the unit.

20. A structural unit as defined by claim 14, characterized by the inseparable union being an integral formation with the remainder of the unit.

EDWARD R. POWELL.